

## UNITED STATES PATENT OFFICE

2,484,540

## LEAD COATING PROCESS

Irving P. Whitehouse, South Euclid, Ohio, assignor to Republic Steel Corporation, Cleveland, Ohio, a corporation of New Jersey

No Drawing. Application October 3, 1945,  
Serial No. 620,176

4 Claims. (Cl. 204—36)

1

The present invention relates to the art of coating metal articles with lead and is particularly concerned with a new method of making lead coated articles which are substantially free from porosity or pin-holes in the coating and are highly resistant to corrosion of the underlying metal.

Electrolytic deposits of lead on ferrous metal articles have been used heretofore to protect such articles against corrosion but the protection realized has not been found to be entirely satisfactory. In general, it may be said that the ferrous metal was corroded in small isolated areas and that the service life was much shorter than was desired when relatively heavy coatings were employed.

It is well known that the cause of such short life and such localized corrosion is traceable to discontinuities in the lead coating generally in the form of pin-holes or pores and that when such pin-holes are closed the underlying ferrous metal is protected against corrosion over substantially its entire coated surface for much longer periods of time.

The present invention provides a new method of making electrolytic lead coatings which are substantially free from pin-holes and its use provides lead coatings which will prevent corrosion of the underlying metal for at least twice as long in accelerated corrosion tests as the prior electrolytic lead coatings of the same thickness. Stated briefly, the present invention comprises the important step of burnishing an electrolytic lead coating in a liquid having lubricating qualities.

Lead may be deposited electrolytically on ferrous metal by several well known procedures. One such procedure is as follows: Ferrous metal is degreased by treating it with a suitable organic solvent, for example, trichlorethylene or carbon tetrachloride, after which the metal is electrolytically cleaned in an alkaline cleaner. Here the metal may be made the anode, cathode, or alternately anode and cathode in the electrolyte. Current density of from 20 amps. to 40 amps. per sq. ft. may be used while the electrolyte temperature is between 180° F. and 200° F. After completion of this electrolytic cleaning the metal is ordinarily rinsed or scrubbed in water to remove oil smut and the like from its surfaces which sometimes are present when the metal was not adequately degreased in the organic solvent. Then the metal is usually given a short acid pickle, for example, in an aqueous bath containing from 8% to 10% by weight of sulfuric acid and at a temperature

2

of 165° F. to 180° F. Ordinarily only a few seconds are required for this pickling operation but longer times may be necessary where heavy scale is present on the metal. Then the metal is again rinsed and scrubbed to remove foreign material from the surface thereof and is immediately immersed in the plating tank so as to prevent oxidation so far as possible.

One well known plating solution is an aqueous electrolyte containing about 64 oz. of lead sulfamate per gallon and about 1.35 oz. per gallon of an addition agent. In still plating with such an electrolyte the bath temperature may range from 100° F. to 110° F. with a current density of from 20 amps. to 40 amps. per sq. ft., the pH value of the bath being maintained between 1.7 and 2.0.

Frequently another step is included between the foregoing pickling and lead plating steps. In 20 this additional step the clean and pickled metal is given a flash coating of electrolytic copper before it is electroplated with lead. This copper coating may approximate 10-millionths of an inch in thickness and may be made from an aqueous electrolyte containing, per gallon, about 2 oz. of cuprous cyanide, about 4 oz. of sodium cyanide, and about 2 oz. of potassium hydroxide, the temperature of the electrolyte being maintained at between 135° F. and 150° F. and current 25 densities of from 20 amps. per sq. ft. to 30 amps. per sq. ft. being used. After the article is so plated with copper it is rinsed with water, and is then electrolytically plated with lead as previously described.

35 The article coated with electrolytic lead, and whether embodying the copper flash coating or not, is rinsed with water and immersed immediately in an alkaline chromate solution for from 5 to 10 seconds. A suitable chromate solution 40 consists of water containing about 10% by weight of sodium chromate and about 1% by weight of sodium hydroxide. Then the article is again rinsed in water, which is preferably hot to expedite drying, or it may be immersed in acetone or 45 alcohol for two or three seconds and then exposed to air where it dries rapidly.

Lead fluoborate electrolytes are also commonly used instead of the lead sulfamate electrolyte above described. When such lead electrolytes are 50 used they may be aqueous solutions containing, per gallon, about 40 oz. of lead fluoborate, about 3 oz. boric acid, about 4 or 5 oz. of free fluoboric acid and about .04 oz. of an additional agent such as bone glue. The current density ranges between about 20 amps. and about 40 amps. per sq.

ft. and the bath temperature is about 100° F. and its pH value is from 1 to 1.5 for still plating.

However the electrolytic coating of lead is formed, whether by one or the other of the foregoing methods or some other method, the lead coated article according to the present invention is then burnished in a lubricant. Preferably, rolls which are covered with cloth or other soft fibrous material are rotated rapidly while being pressed against the electrolytic lead coating and while a mineral or vegetable oil is in contact with the lead.

In general it may be said that any natural or synthetic liquid possessing some lubricating qualities may be used in carrying out this invention, including mineral oils, vegetable oils and synthetic lubricants such as lecithin or containing lecithin.

I am not certain as to exactly what takes place during this burnishing operation but I believe that the burnishing rolls wipe the lubricant into the pores of the lead coating and additionally wipe the surfaces of the lead in such a way as to close the pin-holes whether they actually contain lubricant or not. However, lead coatings treated in this manner have been found to be substantially free from pin-holes and to be quite resistant to corrosion and to withstand accelerated corrosion tests on the order of twice as long as electrolytical coatings not so treated.

Apparently both the burnishing action and the presence of lubricant are important in obtaining the desired results for neither merely dipping the electrolytically coated article in the same lubricant nor burnishing in the absence of lubricant showed any appreciable improvement in corrosion resistance. However, when the burnishing was carried out in the presence of lubricant the rate and extent of corrosion was greatly reduced as evidenced by the extended service life.

Having thus described the invention so that others skilled in the art may be able to understand and practice the same, I state that what I desire to secure by Letters Patent is defined in what is claimed.

What is claimed is:

1. The process of lead coating a metal article which comprises the steps of electrodepositing a coating of lead on such an article and closing pin holes in the coating and increasing the resistance of the article to corrosion by frictionally wiping said coating with soft, fibrous material while the coating is in a mineral oil.

2. The process of lead coating a metal article which comprises the steps of electrodepositing a coating of lead on such an article and closing pin holes in the coating and increasing the resistance of the article to corrosion by frictionally wiping said coating with soft, fibrous material while the coating is in a vegetable oil.

3. The process of making a lead coated metal article which comprises the steps of electrodepositing a coating of lead on the clean surface of such an article and closing pin holes in the coating and increasing the resistance of the article to corrosion by frictionally wiping said coating with soft fibrous material while the coating is in a liquid lubricant.

4. The process of making a lead coated metal article which comprises the steps of electrodepositing a coating of lead on the clean surfaces of such an article and closing pin-holes in the coating and increasing the resistance of the article to corrosion by frictionally wiping the surface of the coating with cloth while the coating is in a liquid lubricant.

IRVING P. WHITEHOUSE.

#### REFERENCES CITED

The following references are of record in the file of this patent:

#### UNITED STATES PATENTS

| Number    | Name          | Date          |
|-----------|---------------|---------------|
| 685,211   | Kennedy       | Oct. 22, 1901 |
| 1,580,198 | Harrison      | Apr. 13, 1926 |
| 1,869,041 | Bengston      | July 26, 1932 |
| 2,126,578 | Roemer et al. | Aug. 9, 1938  |
| 2,141,382 | Ferm          | Dec. 27, 1938 |
| 2,177,316 | Giles         | Oct. 24, 1939 |
| 2,318,592 | Cupery        | May 11, 1943  |

#### FOREIGN PATENTS

| Number  | Country       | Date          |
|---------|---------------|---------------|
| 2,460   | Great Britain | 1881          |
| 130,302 | Great Britain | 1919          |
| 484,103 | Great Britain | 1938          |
| 639,701 | France        | Mar. 17, 1908 |

#### OTHER REFERENCES

Protective Coatings for Metals, by R. M. Burns and A. E. Schuh, published by Reinhold Publishing Co., New York, 1939, pp. 34, 207, 208.

Iron Age, Apr. 30, 1942, pp. 29-44.